

# UNITED STATES PATENT OFFICE.

A. D. BOWMAN, OF NEW YORK, N. Y.

## COMPOUND FOR MAKING WRITING-INK.

Specification forming part of Letters Patent No. **59,549**, dated November 13, 1866.

*To all whom it may concern:*

Be it known that I, A. D. BOWMAN, of the city of New York, in the county and State of New York, have invented a new and useful Compound for Making Writing-Ink; and I do hereby declare that the following is a full, clear, and exact description of the same.

My invention consists in a compound composed of extract of logwood, bichromate of potash, and prussiate of potash, the same to be mixed with water or other suitable liquid for making writing-ink.

The compound is composed of the following ingredients, in about the proportions specified: extract of logwood, thirty-two (32) parts; bichromate of potash, six (6) parts; prussiate of potash, one (1) part.

These ingredients are carefully pulverized in any proper way, and then mixed together and shaken, so that a thorough commingling will

take place. The compound may then be done up in any appropriate way for the market.

In making ink with the compound I find that if five hundred and eighty-five (585) grains be put into one (1) gallon of water an excellent ink of a consistency to flow freely from the pen will be produced.

By this invention a compound can be furnished to the market which will enable all persons to make their own ink expeditiously and without trouble, and at little cost.

What I claim as my invention, and desire to secure by Letters Patent, is—

A compound for making writing-ink, composed of the ingredients substantially as herein specified.

A. D. BOWMAN.

Witnesses:

M. M. LIVINGSTON,  
CHAS. MORRILL.